

# United States Patent Office

3,186,787

Patented June 1, 1965

1

3,186,787

## PROCESS FOR DYEING OR PRINTING SHAPED STRUCTURES OF LINEAR AROMATIC POLYESTERS, ESPECIALLY POLYETHYLENE TEREPHTHALATES

Helmut Gies, Hofheim, Taunus, and Wilhelm Happe, Schwalbach, Taunus, Germany, assignors to Farbwurke Hoechst Aktiengesellschaft vormals Meister Lucius & Brüning, Frankfurt am Main, Germany, a corporation of Germany

No Drawing. Filed Dec. 17, 1962, Ser. No. 244,933  
Claims priority, application Germany, Dec. 27, 1961,

F 35,668

4 Claims. (Cl. 8-41)

The present invention relates to a process for dyeing or printing shaped structures of linear aromatic polyesters, especially polyethylene terephthalates.

We have found that fast yellow dyeings and prints can be produced on shaped structures of aromatic polyesters, especially polyethylene terephthalates, such as filaments, tapes, fabrics, fibers or threads produced from fibers, by treating the shaped structures at an elevated temperature with an aqueous dispersion of the disazo-dyestuff of phenol-(4 azo 1)-benzene-(4 azo 4)-phenol having the formula



The dyeing is carried out in the presence of a carrier at a temperature within the range of about 95° to 105° C. and preferably about 100° C. or, by the high temperature process, in the absence of a carrier at a temperature within the range of about 120° to 140° C. and preferably between about 125° and 130° C. Printing is advantageously carried out by applying the dispersed dyestuff to the shaped structures by printing and subjecting the printed shaped structure to a short dry heat treatment at a high temperature, for example, of about 200° C.

As carriers which are suitable for the process of the present invention there may be used, for example, o- or p-phenyl phenol, salicylic acid esters, methyl salicylic acid esters, mono-, di- and trichlorobenzenes, benzoic acid and methyl naphthalene. In order to improve the fastness to abrasion, the dyeings or prints produced according to the process of the present invention may be after-treated in an alkaline reducing bath which may contain, for example, sodium dithionite, sodium hydroxide and a detergent.

The dyestuff shows a good affinity to structures of aromatic polyesters and a good ability of building up, even when dyeing at 100° C. in the presence of carriers. The dyeings obtained are distinguished by their excellent fastness to light and their very good fastness to thermo-fixation.

The following examples serve to illustrate the invention but they are not intended to limit it thereto, the parts being by weight unless otherwise stated and the relationship of parts by weight to parts by volume being the same as that of the kilogram to the liter.

### Example 1

100 grams of yarn of polyethylene terephthalate are treated for 90 minutes at a goods-to-liquor ratio of

2

1:30 in a bath of 100° C. containing 0.8 gram of the disazo-dyestuff of phenol-(4 azo 1)-benzene-(4 azo 4)-phenol in a finely divided form and 4 grams per liter of a carrier based on o-phenyl phenol. The goods are soaped and then subjected to an after-treatment for 15 minutes at 80° to 90° C. in a reducing bath containing per liter 2 grams of sodium dithionite 2 ml. of sodium hydroxide solution of 38° Bé, and 0.5 to 1 gram of a non-ionic synthetic detergent (polyglycol ether) in order to improve their fastness to rubbing. There is obtained a reddish yellow dyeing possessing a very good fastness to light and to thermofixation.

### Example 2

100 grams of a fabric of polyethylene terephthalate are treated for 90 minutes at a goods-to-liquor ratio of 1:20 in a bath of 120° C. containing 0.4 gram of the disazo-dyestuff of phenol-(4 azo 1)-benzene-(4 azo 4)-phenol in a finely divided form. The goods are subjected to an after-treatment in a reducing bath as described in Example 1. There is obtained a reddish yellow dyeing possessing the same good fastness properties as described in Example 1.

### Example 3

25 100 grams of a fabric of polyethylene terephthalate are printed with a printing paste containing per kilogram 50 grams of the disazo-dyestuff of phenol-(4 azo 1)-benzene-(4 azo 4)-phenol, 200 grams of nafka rubber, 50 grams of naphtholdiglycol ether and 700 grams of water. The goods are then dried, fixed for 30 seconds at 200° C. and finally subjected to an after-treatment in a reducing bath as described in Example 1. There is obtained a yellow print possessing good fastness properties.

35 We claim:

1. A process for dyeing and printing fibrous materials of polyethylene terephthalates, which comprises applying to said materials at about 95 to 140° C. from an aqueous dispersion the disazo dyestuff phenol-(4 azo 1)-benzene-(4 azo 4)-phenol of the formula



45 2. The process as claimed in claim 1, wherein the dyeing is carried out in the presence of a carrier at a temperature between about 95° and 105° C.

50 3. The process as claimed in claim 1, wherein the dyeing is carried out in the absence of a carrier at a temperature between about 120° and 140° C.

40 4. The process as claimed in claim 1, wherein the printed fibrous materials are exposed to a short dry heat treatment at about 200° C.

### References Cited by the Examiner

#### UNITED STATES PATENTS

|           |       |                    |
|-----------|-------|--------------------|
| 2,663,612 | 12/53 | Gibson.            |
| 2,881,045 | 4/59  | Mecco et al.       |
| 2,926,987 | 3/60  | Freyermuth et al.  |
| 2,934,397 | 4/60  | Landerl.           |
| 3,096,140 | 7/63  | Gaetani ----- 8/41 |

NORMAN G. TORCHIN, Primary Examiner.